# EUROPEAN PATENT SPECIFICATION

(11) **EP 0 024 198 B1**
(45) Date of publication and mention of the grant of the patent: **26.09.1984**
(21) Application number: 80302786.1
(22) Date of filing: 13.08.1980
(51) Int. Cl.: D02G 3/22

(54) **Mixed fiber length yarn**
Garn aus Fasern unterschiedlicher Länge
Fil issu de fibres de longueurs différentes

(30) Priority: 13.08.1979 US 66216
(43) Date of publication of application: 25.02.1981
(73) Proprietor: CELANESE CORPORATION, New York New York 10036 (US)
(72) Inventor: Sawyer, Linda C., Chatham New Jersey (US)
(74) Representative: Beton, John Lonsdale

## Description

The present invention relates to yarns comprising polyester staple fibers, especially novel yarns comprised of polyester fibers having different lengths. For many years natural fibers such as cotton and wool have been replaced, either wholly or in a part, by synthetic fibers, especially polyester fibers, in the manufacture of yarns and fabrics. Significant improvements in the strength and processability of textile yarns have thus been achieved. Synthetic fiber-containing yarns and fabrics do not, however, typically possess the appearance and physical characteristics of cotton or wool yarns and fabrics. Synthetic fiber-containing fabrics also do not generally attain the same level of comfort as natural fiber-containing fabrics.

Attempts have thus been made to improve the physical characteristics of synthetic fiber-containing yarns and fabrics. For example US Patent 3 350 872 describes a textile yarn comprised of synthetic fibers whose physical characteristics are intended to simulate those of a wool fabric, which yarn consists of a crimped and uncrimped acrylic fiber. US Patent No 3 965 664 describes a yarn which has the feel of a natural fiber-containing yarn. The yarn is formed by blending a mixture of at least three different groups of fibres, the denier of the fibers in each group being different from the denier of the fibers in the other groups. Optionally the length of the fibers in each group may differ from the length of the fibers in the other groups. US Patent 3 188 790 discloses yarns comprised of a blend of synthetic fibers (e.g. nylon or polyethylene terephthalate) and cotton fibers, with the synthetic fibers being both crimped and uncrimped. US Patents 3 587 220 and 3 686 850 disclose yarns comprised of synthetic fibers having high and low shrinkage characteristics. US Patent No. 2 271 184 describes a blend of fibers formed by blending a group of fibers having a substantially uniform denier along their length with a group of fibers having thick and thin portions along their length. Optionally the length of the fibers may vary from 25 to 100%. Differential fiber length is also a criterion taken into account in U.S. Patents 3 157 021; 3 371 475; and 3 335 466 in order to produce a bulky, high strength synthetic yarn. A synthetic fiber-containing yarn has not been produced, however, which adequately exhibits the advantageous physical characteristics (e.g., bulkiness and appearance) of natural fiber-containing yarns while retaining the strength and durability of synthetic fiber-containing yarns.

In one aspect of the present invention there is provided an improved synthetic fiber-containing yarn comprising polyester fibers or a blend of polyester staple and other staple fibers of which at least 50 percent by weight are polyester fibers, the polyester fibers comprising at least 3 groups, wherein the polyester fibers in each of said groups have a substantially uniform length such that the fiber lengths within each group differ by a factor of 5 percent or less, and wherein the length of polyester fibers in each group differs from the length of polyester fibers present in any other group by a factor of at least 15 percent and wherein the groups are distributed among all of the following ranges:
(a) up to 75 percent by weight of the polyester fibers have a length X, wherein X represents the length of the longest polyester fiber group and has a value of between 1 and 6 inches (2.5 and 16.2 cm).
(b) up to 75 per cent by weight of the polyester fibers have a length greater than 1/2X, but not including said length of about X, and
(c) up to 35 per cent by weight of the polyester fibers have a length less than or equal to 1/2X.

In another aspect of the present invention, there is provided an improved fabric containing such polyester fiber-containing yarn.

A preferred distribution of polyester fibers within the above ranges consists of between 25 and 50 percent by weight of polyester fibers having a length of X, between 25 and 50 percent by weight of polyester fibers having a length greater than 1/2X, but not including said length of about X, and up to 30 percent by weight of polyester fibers having a length less than or equal to said length of 1/2X. Most preferably the yarn contains less than 20 percent by weight of polyester fibers having a length less than or equal to said length of 1/2X.

It has been found that yarns which contain polyester fibers in these lengths and proportions possess characteristics closely paralleling those of natural fiber-containing yarns (e.g., cotton or wool yarns). These characteristics relate to aesthetic factors as well as to the thermal and tactile comfort of fabrics containing such yarns.

Fabrics containing yarns comprised of natural fibers such as cotton generally exhibit "comfort" characteristics which are superior to those exhibited by fabrics which contain conventional polyester fiber-containing yarns. Generally, natural fiber-containing yarns exhibit a greater bulk than polyester yarns (i.e. the yarns consist of loosely packed fibers). Natural fiber-containing yarns consist of a mixture of fibers of differing length, thus providing a yarn having a multitude of protruding ends along the longitudinal axis of the yarn.

The high bulk of natural fiber-containing yarns enables fabrics to be produced which exhibit low air permeability and satisfactory covering characteristics. The high degree of fiber end protrudence also enhances the comfort of the fabric.

The significant degree of protrudence of fiber ends from the yarn in such fabrics provides for greater tactile comfort in comparison to conventional polyester yarn-containing fabrics. Conventional polyester yarns typically consist of fibers having a uniform length, therefore providing a lessened amount of protruding ends resulting in a smoother tactile sensation, high degree of air permeability, and low bulk.

The novel polester fiber-containing yarns and fabrics of the present invention have properties such as drape, bulk and porosity which more nearly simulate those of natural fiber-containing yarns and fabrics, while additionally exhibiting the strength and durability of polyester fiber-containing yarns.

The yarns of this invention contain at least three groups of polyester fibers with the polyester fibers within each group being of substantially the same length. It is recognized that the fiber lengths within each group will normally not be exactly the same due to the lack of precision which exists when large amounts of such fibers are cut, but the fiber lengths within each group will generally only differ by a factor of 5 percent or less. For example, if the longest length X of the polyester fibers in the groups is intended to be 3 inches (7.6 cm), the group of fibers which is cut to that length will generally contain polyester fibers differing from the desired 3 inch (7.6 cm) length by a factor of plus or minus 5 percent or less. This group of fibers will, for purposes of the invention, be deemed to contain fibers of 3 inches (7.6 cm) in length (i.e. a length of X). Similarly, the term "1/2X" is intended to include lengths of 1/2X plus or minus 5 percent. That is, if the longest length X of the synthetic fibers in the groups is intended to be 3 inches, then fibers having a length of 1/2X will differ from a length of 1 1/2 inches (3.8 cm) by only plus or minus 5 percent.

The substantially uniform length of the polyester fibers of each of the groups present in the yarn will also differ from the substantially uniform length of the polyester fibers in the other groups present in the yarn by at least 1 percent and preferably between 1 5 percent and 30 percent in order to provide a uniform and high degree of fiber end protrudence along the longitudinal axis of the yarn.

The polyester fibers within the yarn must consist of a minimum of three groups of polyester fibers in order to obtain the desired characteristics. More than three groups of polyester fibers may be present as long as the lengths of all of the fibers present in the yarn are distributed in the required proportions. However, yarn production considerations (e.g., the problems which arise from handling multiple lengths of fibers) discourage the use of an excessive number of groups of polyester fibers of differing lengths. The advantages of the present invention may generally be achieved by employing anywhere from three to six groups of polyester fibers of such lengths and in such proportions consistent with the required distribution of the polyester fibers within the yarns of this invention.

In order to attain the full benefit of the yarn of the present invention, each of the groups of polyester fibers contained in the yarn should be present in a significant amount. That is, each group should preferably comprise at least 5 percent by weight of the total weight of the polyester fibers contained within said groups. However, the percentage of polyester fibers in any group may be less than 5 percent by weight in certain instances, such as when more than three groups of polyester fibers are present in the yarn. For example one polyester yarn made according to the invention contained six groups of fibers of different lengths ranging from 1-1/2 inches (3.8 cm) to 1/4 inch (0.6 cm) as follows:-
19.4% by weight of fibers having a length of inches (3.8 cm).
41.7% by weight of fibers having a length of t inches (3.2 cm).
30.4% by weight of fibers having a length of 1 inch (2.5 cm).
12.5% by weight of fibers having a length of inch (1.9 cm).
4.6% by weight of fibers having a length of inch (1.3 cm).
1.4% by weight of fibers having a length of inch (0.6 cm).

The different fiber lengths to be used within the groups present in the yarn can vary greatly depending upon the desired yarn characteristics as well as the intended use of the yarn. For example, textile fabrics whose primary use is in shirts and similar wearing apparel typically will be comprised of a yarn which contains polyester fibers having a longest length of about 1 t inches (3.8 cm). Yarns which are to be used in the production of sweaters, however, will typically contain polyester fibers having a longest length of 3 (7.6 cm) to 6 inches (15.2 cm). The determination of the longest length to be used in a yarn which is intended for a specific use is well within the skill of the artisan.

Thus, in accordance with the required fiber distribution of the present invention, a yarn whose primary use lies in the shirting field could contain up to 75 percent by weight of polyester fibers of 1 t inches (3.8 cm) in length, up to 75 percent by weight of polyester fibers having a length greater than 4 of an inch (1.9 cm) and up to 35 percent by weight of polyester fibers having a length less than or equal to said length of t of an inch (1.9 cm), based upon the weight of the fibers in those three groups.

The polyester fibers in each of the above ranges may be provided by more than one group of fibers, with the substantially uniform length of the polyester fibers of one group differing from the substantially uniform length of the polyester fibers of the other group by a factor of at least 15 per cent. However, the total weight percentage of the polyester fibers in the group must not exceed the allowable proportion for fibers of those lengths.

For example, in a yarn which contains 50 percent by weight of polyester fibers of 1 t inches (3.8 cm) in length, 40 percent by weight of polyester fibers having a length greater than 4 of an inch (1.9 cm) and 10 percent by weight of polyester fibers having a length less than or equal to said length of of an inch (1.9 cm) (based upon the weight of the fibres in those groups), the polyester fibres having a length of between and inches (1.9 and 3.8 cm) could be evenly distributed between fibers 1 inch (2.5 cm) in length and fibers 1 t inches (3.2 cm) in length (i.e., 20 percent by weight of each based on the total weight of the synthetic fibers present).

It should be understood that the length of the longest polyester fibers to be used in the groups contained within the novel yarn of this invention may be much greater than 1 t inches (3.8 cm), and may indeed be 3 to 6 inches (7.6 or 15.2 cm) in length. However, the minimum length of the fibers present will necessarily be more closely controlled, since it may become very impractical to incorporate any fiber length of less than 1 inch (0.6 cm) in length into the yarn during the production sequence. The shortest length of any polyester fibers present will thus generally be at least t inch (1.3 cm).

The production of a polyester fiber-containing yarn which contains polyester fibers of lengths which vary over a wide range may also present problems during the production of the yarn. It is thus also advantageous to employ groups of polyester fibers which have significantly differing lengths but which lengths do not differ too greatly. For example, a yarn containing polyester fibers having lengths of 3 inches (7.6 cm), 1 t inches (4.4 cm), and of an inch (1.9 cm) would be acceptable both with respect to length differential among the groups as well as the minimum length present.

A most preferred distribution of polyester fibers within a yarn contains 20 percent by weight of polyester fibers of 1 t inches (3.2 cm) in length, 40 percent by weight of polyester fibers having a length of 1 inch (2.5 cm), 25 percent by weight of polyester fibers having a length of of an inch (1.9 cm) and 15 percent by weight of polyester fibers having a length of t of an inch (1.3 cm).

Other physical characteristics of the polyester fibers used in the novel yarns of this invention may be varied in order to further increase the overall bulk of the yarn. For example, at least a portion of the polyester fibers may be crimped prior to being incorporated into the yarn. Mixtures of shrinkable and non-shrinkable polyester fibers may also be used to increase yarn bulk. At least a portion of the polyester fibers may also have an irregularly-shaped or non-circular cross-section. Fibers of mixed deniers may also be used with the yarns of the present invention.

The polyester fibers present in the yarn comprise at least 50 percent by weight of the total fibers present in the yarn and consist of a mixture of at least three groups of polyester fibers of substantially uniform length, with the polyester fibers contained within the at least three groups being present in the required proportions in order to ensure that the benefits of the present invention are attained. Preferably, the polyester fibers contained within the at least three groups are present in the yarn in amounts ranging from about 65 to 100 percent by weight based on the total weight of the fibers present in the yarn.

The yarns of this invention may also contain natural fibers such as cotton or wool fibers in conventional weight ratios which typically range from 50:50 to 90:10 polyester fiber/natural fiber, with preferred ratios being 65:35 and 80:20. It should be noted, however, that when the yarn contains both polyester and natural fibers, the natural fibers need not be present in the required number of groups of the specified ranges set forth for the polyester fibers. In addition, the yarn of this invention may also contain synthetic fibers other than polyester fibers, such as rayon or nylon, instead of or in mixture with the natural fibers. Thus, for example, the yarn could comprise 65% mixed length polyester and 35% rayon or nylon.

The novel polyester fiber-containing yarns of this invention may be formed into novel fabrics which exhibit improved comfort characteristics as compared to conventional polyester fiber-containing fabrics. The fabrics may be produced by conventional processes (e.g. by knitting or weaving). Due to the increased bulk and protruding end count of the novel yarns of this invention, fabrics produced therefrom will exhibit improved covering characteristics as well as an improved tactile sensation. Such fabrics will therefore more closely possess the "look and feel" of natural fiber-containing fabrics, such as cotton and wool fabrics.

Fabrics may also be prepared which comprise a mixture of the novel polyester fiber-containing yarns of the present invention and conventional natural fiber-containing yarns of synthetic fiber-containing yarns. The novel yarns of this invention may be blended with such natural or synthetic fiber-containing yarns in conventional weight ratios.

The yarns of this invention may be produced in any conventional manner. Any desired blending, carding, drafting and spinning sequence may be used to produce the yarns. When it is initially determined what distribution of polyester fiber lengths is desired in the yarn to be produced, groups of polyester fibers are cut on a cutting wheel set to the appropriate lengths. The cut fibers are then blended and carded whereupon the various lengths become randomly distributed. The yarn which is then spun from the mixture of fibers will contain the specified lengths of polyester fibers in the required proportions. The fibers of each of the groups become randomly distributed and dispersed throughout the yarn during the yarn production process and are not actually grouped or segregated as to fiber lengths within the yarn which is produced.

The following experiments illustrate but do not limit the invention. Four yarns were prepared as set forth in Table I.

Fabrics prepared from each of the yarns A, B, C and D were tested using a Mitex Bending Tester to determine the bending rigidity of the yarns from which they were prepared. The bending rigidity of a yarn is indicative of how a fabric or garment containing that yarn will drape or hang from a person. The relative softness of a fabric is related to the bending rigidity of the yarn within the fabric, with a high value for bending rigidity being indicative of a high degree of fiber end protrudence within the yarn since the presence of protruding ends provides frictional resistance to bending.

Table II sets forth the bending rigidity for the various yarns identified above.

As may be seen from the above data, the cotton yarn exhibits the highest bending rigidity of the yarns tested. However, the mixed fiber length yarn which falls within the scope of the present invention (yarn D) exhibits a bending rigidity which is greater than that exhibited by any of the yarns except the cotton yarn. It is noted that the bending rigidity of the polyester mixed fiber length yarn is significantly greater than the bending rigidity of the conventional polyethylene terephthalate yarn (i.e. yarn A).

The fabrics prepared from yarns A, B, C and D were further tested to determine certain other of their characteristics as set forth below:

The above data shows that a fabric produced from a yarn comprising polyester fibers of mixed fiber length according to the present invention (i.e. yarn D) exhibits a bulk area (i.e. a measure of yarn bulk including loops and hairs) which is greater than the bulk area of a cotton fabric produced from a conventional cotton yarn (i.e. yarn B). The bulk area measurements of Table III were made on a Quantimet 720 Image Analyzing Computer and constitute the average of over fifty measurements. The bulk area of the fabric produced from the mixed fiber length yarn of the present invention is significantly greater than the bulk area of the fabric produced from a conventional polyester yarn (i.e. yarn A). Therefore, the fabric produced from yarn D, while having a thickness and weight that are not excessive, exhibits a significant increase in bulk area which is highly desirable since the bulk area of a fabric is directly related to the coverage to be afforded by that fabric per unit weight. That is, an increase in the bulk area of a fabric will result in an increase in the covering characteristics of the fabric.

In addition, fabrics produced from the yams comprising fibers of mixed fiber length according to the present invention exhibit a water vapor transmission rate (WVTR) which is significantly lower than that exhibited by conventional synthetic fabrics while also approaching the values for cotton fabrics. The water vapor transmission rate is defined in accordance with ASTM test 896-66 and is indicative of the amount of water vapor which passes through a unit area of fabric per unit time at a vapor pressure difference of about 6.6 mm Hg at 70°F (21 °C) and 65 percent relative humidity.

The water vapor transmission rate of a fabric is indicative of the relative porosity and the covering characteristics of the fabric. That is, a fabric comprised of a yarn having a large number of protruding ends will necessarily be less porous than a fabric comprised of a yarn having a lesser number of protruding ends.

## Claims

1. A yarn comprising polyester staple fibers or a blend of polyester staple and other staple fibers of which at least 50 percent by weight are polyester fibers, the polyester fibers comprising at least 3 groups, wherein the polyester fibers in each of said groups have a substantially uniform length such that the fiber lengths within each group differ by a factor of 5 percent or less, and wherein the length of polyester fibers in each group differs from the length of polyester fibers present in any other group by a factor of at least 15 percent and wherein the groups are distributed among all of the following ranges:
(a) up to 75 percent by weight of the polyester fibers have a length X wherein X represents the length of the longest polyester fiber group and has a value of between 1 and 6 inches (2.5 and 16.2 cms).
(b) up to 75 percent by weight of the polyester fibers have a length greater than tx, but not including said length of about X, and
(c) up to 35 percent by weight of the polyester fibers have a length less than or equal to ZX.

2. A yarn according to claim 1 wherein each group of polyester fibers is present in an amount of at least 5 percent by weight of the total weight of the polyester fibers.

3. A yarn according to claim 1 wherein the length X has a maximum value of 1 t inches (3.8 cm) and wherein any other staple fibers present in said yarn are cotton.

4. A yarn according to claim 3 wherein the groups are distributed among the following ranges:
(a) between 25 and 50 percent by weight of the polyester fibers have a length X,
(b) between 25 and 50 percent by weight of the polyester fibers have a length greater than but not including said length of about X, and
(c) between 5 and 30 percent by weight of the polyester fibers have a length less than or equal to tx polyester.

5. A yarn according to claim 3 wherein said polyester fibers consists of three to six groups.

6. A fabric containing the yarn of claim 1.

7. A fabric containing the yarn of claim 3.

8. A fabric containing the yarn of claim 4.

## Revendications

1. Fil comprenant des fibres discontinues en polyester ou un mélange de fibres discontinues en polyester et d'autres fibres discontinues dont au moins 50 % en poids sont des fibres de polyester, les fibres de polyester comprenant au moins trois groupes, où les fibres de polyester de chacun desdits groupes ont une longueur sensiblement uniforme telle que les longueurs des fibres de chaque groupe diffèrent d'un facteur de 5 % ou moins, et où la longueur des fibres de polyester de chaque groupe diffère de la longueur des fibres de polyester présentes dans tout autre groupe d'un facteur d'au moins 15%, et où les groupes sont distribués parmi toutes les plages suivantes:
(a) justu'à 75 % en poids des fibres de polyester ont une longueur X, où X représente la longueur du plus long groupe de fibres de polyester et possède une valeur comprise entre 2,5 et 16,2 cm (1 et 6 inches),
(b) jusqu'à 75 % en poids des fibres de polyester ont une longueur supérieure à X/2, mais non compris ladite longueur d'environ X, et
(c) jusqu'à 35 % en poids des fibres de polyester ont une longueur inférieure ou égale à X/2.

2. Fil selon la revendication 1, dans lequel chaque groupe de fibres de polyester est présent en quantité d'au moins 5 % en poids du poids total des fibres de polyester.

3. Fil selon la revendication 1, dans lequel la longueur X présente une valeur maximale de 3,8 cm (1,5 inch) et dans lequel toutes autres fibres discontinues présentes dans ledit fil sont en coton.

4. Fil selon la revendication 3, dans lequel les groupes sont distribués parmi les plages suivantes:
(a) entre 25 et 50 % en poids des fibres de polyester ont une longueur X,
(b) entre 25 et 50 % en poids des fibres de polyester ont une longueur supérieure à X/2, mais non compris ladite longueur d'environ X, et
(c) entre 5 et 30 % en poids des fibres de polyester ont une longueur inférieure ou égale à X/2.

5. Fil selon la revendication 3, dans lequel lesdites fibres de polyester comprennent trois à six groupes.

6. Etoffe contenant le fil de la revendication 1.

7. Etoffe contenant le fil de la revendication 3.

8. Etoffe contenant le fil de la revendication 4.

## Patentansprüche

1. Garn, bestehend aus Polyesterstapelfasern oder einem Gemisch von Polyesterstapelfasern und anderen Stapelfasern, bei welchem mindestens 50 Gew.-% aus Polyesterfasern bestehen, wobei die Polyesterfasern mindestends 3 Gruppen umfassen, die Polyesterfasern in einer jeden Gruppe eine im wesentlichen gleichförmige, nur um einen Faktor von höchstens 5% differierende Länge aufweisen, die Länge der Polyesterfasern in einer jeden Gruppe von der Länge der Polyesterfasern in jeder anderen Gruppe um einen Faktor von mindestens 15 % differiert und die Gruppen in die folgenden Bereiche fallen:
(a) bis zu 75 Gew.-% der Polyesterfasern haben eine Länge X, wobei X die Länge der längsten Polyesterfassergruppe bedeutet und einen Wert zwischen 1 und 6 Inch (2,5 und 16,2 cm) besitzt,
(b) bis zu 75 Gew.-% der Polyesterfasern eine Länge von mehr als 1/2X haben, wobei diejenigen mit einer Länge von ungefähr X nicht eingeschlossen sind, und
(c) bis zu 35 Gew.-% der Polyesterfasern eine Länge von 1/2X oder weniger haben.

2. Garn nach Anspruch 1, bei welchem jede Gruppe von Polyesterfasern mindestens 5 Gew.-% des Gesamtgewichts der Polyesterfasern ausmacht.

3. Garn nach Anspruch 1, bei welchem die Länge X einen Mindestwert von 1 1/2 Inch (3,8 cm) besitzt und bei welchem andere eventuell vorhandene Stapelfasern im Garn aus Baumwolle bestehen.

4. Garn nach Anspruch 3, bei welchem die Gruppen in die folgenden Bereiche fallen:
(a) zwischen 25 und 50 Gew.-% der Polyesterfasern haben eine Länge X,
(b) zwischen 25 und 50 Gew.-% der Polyesterfasern haben eine Länge von mehr als 1/2X, wobei diejenigen mit einer Länge von ungefähr X nicht eingeschlossen sind, und
(c) zwischen 5 und 30 Gew.-% der Polyesterfasern haben eine Länge 1/2X oder weniger.

5. Garn nach Anspruch 3, bei welchem die Polyesterfasern aus drei bis sechs Gruppen bestehen.

6. Textilstoff, der das Garn nach Anspruch 1 enthält.

7. Textilstoff, der das Garn nach Anspruch 3 enthält.

8. Textilstoff, der das Garn nach Anspruch 4 enthält.
